

Aug. 19, 1930.

W. E. B. BAKER

1,773,419

SULPHITE WOOD PULP AND METHOD OF MAKING THE SAME

Filed June 3, 1926



WITNESS:

Bob R. Kitchel.

INVENTOR

Webster E. Byron Baker

BY

Augustus B. S. Wiegert.

ATTORNEY.

## UNITED STATES PATENT OFFICE

WEBSTER E. BYRON BAKER, OF BROOKLYN, NEW YORK

## SULPHITE WOOD PULP AND METHOD OF MAKING THE SAME

Application filed June 3, 1926. Serial No. 113,408.

The principal objects of the present invention are to increase the yield and improve the quality and strength of unbleached sulphite pulp suitable for making wrapping and bag paper; to improve the fibers; to shorten the sulphite cooking period; and to provide an economical and effective process for obtaining the foregoing objects.

Stated generally, the invention consists in 10 treating wood chips with alkali solutions adapted to render their alpha lignin insoluble in bisulphite cooking liquor before digesting the chips in bisulphite cooking liquor.

The invention also comprises rendering 15 the alpha lignin insoluble in the subsequent step of cooking with bisulphite acid solution by treating the wood chips with an alkali solution containing or consisting of free acting ammonia which, augmenting the vapor 20 pressure at the temperature employed in the digester, forces the alkali solution into the pores of the chips.

The invention also comprises sulphite pulp 25 characterized by abnormally high lignin content and by the strength and flexibility of its fibers.

The invention also comprises the improvements to be presently described and finally claimed, and in the following description 30 reference will be made to the accompanying drawing forming part hereof and in which the single figure, more or less diagrammatically, illustrates one form of apparatus in connection with which the invention may be 35 practiced.

In the drawing 1, 2 and 3 are digesters of the general type used in making sulphite wood pulp from wood chips by cooking them with bisulphite liquor. Each digester is fitted with steam connections 4 leading to the top and bottom and provided with valves and also with valved blow off or discharge connections 5, and also with valved connections 6 for bisulphite cooking acid, and also 40 with valved relief connections 7 for air, sulphurous acid gas or vapor,  $\text{SO}_2$ , and bisulphite cooking acid. There is nothing new involved in the apparatus above described. There are means for introducing and withdrawing weak alkali solutions to and from the 45 digesters. As shown these means comprise a closed receptacle 8 in a closed valved pipe circuit 9, which includes a pump 10 and which communicates by valved branches 11 with the digesters, and there is also a valved connection 12 between each of the digesters. 55

The method or improvement of the invention may be described in connection with the apparatus above referred to as follows:

In the description reference will be made 60 at first to one digester, for example 3. The digester is properly supplied with wood chips and the chips are subjected to weak alkali solution and steam by way of the connections 4 and 11. The result of this is that alpha lignin is rendered insoluble in the cooking acid employed at a later stage of the process and in the usual way. An example of weak alkali solutions are solutions of caustic soda, 65 barium hydrate and the like. A descriptive but not limiting example of temperature is 90 to 100° C. more or less and as a descriptive, 70 but not limiting, example of an alkali solution adapted to render alpha lignin insoluble in the subsequent cooking step, reference may be made to one differing only by a few hundredths specific gravity departure from water, more or less. Stronger solutions of alkali effect economy in time at the expense of economies in chemical consumption. The 75 duration or length of the treatment varies, but descriptively reference may be made to one or two hours. The described treatment of the wood chips in the digester may well be carried on in the presence of ammonia 80 which, creating relatively high vapor pressure at the temperature employed, forces the solution into the pores of the wood. The ammonia can be supplied along with the alkali solution in the manner described or it may be injected into the digester. Upon completion of the described step the alkali solution may be withdrawn by way of the connection 11, or it may be passed by way 85 of the connection 12 into the digester 2 filled with wood chips and used in the treatment of the chips in the digester 2, and in the latter case an economy is effected in that the heat of the alkali solution is imparted to the 90

heat of the alkali solution is imparted to the 100

chips in the digester 2 and is not wasted or lost.

The next step is the well known step of cooking the chips for example in any of the digesters shown, or in any digester with bisulphite liquor or cooking acid which step is too well understood to require detail description. The pulp is finally discharged as at 5 and it of course contains the alpha lignin so that the yield is increased and the fibers are improved by having been subjected to the swelling effect of hydroxyl ions in the first treatment and to the shrinking effect of acid in the second treatment or step.

15 In respect to the step of cooking in acid liquor there are advantages due to the primary treatment of the wood chips in the digester with an alkali solution as described, and among these advantages reference may be made to the fact that the discharge of the weak alkali solution from the digester leaves a partial vacuum which promotes the penetration of the chips by the cooking acid. Resin saponification and elimination from the wood by the weak alkali solution treatment previous to cooking facilitates penetration of the cooking acid into the pores of the chips. The result of these factors is that the sulphite cooking periods are made shorter, thus effecting an economy additional to the economy effected by increased yield while at the same time the quality of the wood pulp is improved in regard to strength, flexibility and otherwise for uses and purposes of which bag and wrapping paper are examples.

It will be obvious to those skilled in the art that modifications may be made in details of procedure and in the choice of the alkali solution or of the original raw material without departing from the spirit of the invention which is not limited in those respects or otherwise than as the prior art and the appended claims may require.

I claim:

45 1. In the manufacture of sulphite wood pulp the improvement which consists in rendering the alpha lignin insoluble in the subsequent step of cooking with bisulphite acid liquor by primarily treating wood chips in a digester with an alkali solution including free acting ammonia which creating relatively high vapor pressure at the temperature employed forces the alkali solution into the pores of the wood.

55 2. In the manufacture of sulphite wood pulp the improvement which consists in establishing a plurality of digesters containing wood chips, primarily treating the wood chips in one digester with alkali solution adapted to render alpha lignin insoluble, transferring the solution while hot from the first digester to a second digester and there treating chips with the hot solution, and introducing bisulphite acid cooking liquor

into the first digester and cooking the chips therein.

3. In the manufacture of sulphite wood pulp the improvement which consists in treating wood chips in a digester with alkali solution adapted to render alpha lignin insoluble in the subsequent step of cooking, discharging the alkali solution from the digester and thereby creating a partial vacuum, and introducing bisulphite cooking liquor and cooking the chips.

4. In the manufacture of sulphite wood pulp the improvement which consists in treating wood chips in a digester with alkali solution including free acting ammonia, removing the solution and thereby creating a partial vacuum, and introducing bisulphite cooking liquor into the partial vacuum and cooking the chips.

5. Sulphite pulp characterized by abnormally high alpha lignin content.

6. Sulphite pulp characterized by abnormally high alpha lignin content and by strength and flexibility of its fibers exceeding that where the beta lignin is present.

7. Sulphite wood pulp containing alpha lignin in a form insoluble in bisulphite acid cooking liquor.

8. Sulphite wood pulp of low resin content and containing alpha lignin in a form insoluble in bisulphite acid cooking liquor.

9. In the manufacture of sulphite wood pulp the improvement which consists in initially preparing the wood chips for cooking by treating them in a digester with alkali solution and limiting the action of the alkali by low temperature and low concentration such that none of the lignin is cooked and the alpha lignin is rendered insoluble in the subsequent step of cooking with bisulphite liquor, and then pulping the so treated chips by cooking them with bisulphite liquor.

10. In the manufacture of sulphite wood pulp the improvement which consists in primarily treating the wood chips in a digester with an alkali solution differing only by a few hundredths specific gravity departure from water to render the alpha lignin insoluble in the subsequent step of cooking with bisulphite liquor, and then pulping the so treated chips by cooking them with bisulphite liquor.

11. A process for manufacturing pulp in two stages of which the first is a treatment of the wood chips with alkali solution differing only by a few hundredths specific gravity departure from water, and of which the second comprises an acid treatment of the chips resulting in the production of pulp.

WEBSTER E. BYRON BAKER.

125

130